

# UNITED STATES PATENT OFFICE.

HUGH RODMAN, OF EDGEWOOD, PENNSYLVANIA, ASSIGNOR TO RODMAN CHEMICAL COMPANY, OF VERONA, PENNSYLVANIA, A CORPORATION OF PENNSYLVANIA.

## METHOD OF CARBURIZING.

1,292,652.

Specification of Letters Patent. Patented Jan. 28, 1919.

No Drawing.

Application filed June 16, 1917. Serial No. 175,235.

To all whom it may concern:

Be it known that I, HUGH RODMAN, a citizen of the United States, and a resident of Edgewood, in the county of Allegheny and 5 State of Pennsylvania, have made a new and useful Invention in Methods of Carburizing, of which the following is a specification.

This invention relates to the carburizing of steel and discloses a new and improved 10 method of maintaining the efficiency of the carburizing material.

Steel is packed with carburizing material in pots or boxes and then subjected to 1500 15 degrees Fahrenheit. When sufficient carbon has been absorbed by the steel the pot is withdrawn from the furnace and then either cooled down or opened up while still hot. In the latter case the carburizing material is liable to burn and lose its carburizing efficiency and therefore it is customary either to cool the material in an air tight receptacle (sometimes the box or pot after the metal parts have been removed) or to 20 quench it with water, generally by sprinkling and raking the material about on the floor till cool enough to resist ignition.

Whether the material is cooled in the boxes without opening them or is exposed hot and afterward cooled in any desired 25 way, the user frequently adds some additional energizer (generally soda ash in the form of a fine powder) to bring the material up to a standard strength. This is done by mixing the used material with a little dry 30 soda ash, the idea being to compensate for the alkali which may have been vaporized during the carburizing heat or which may have been burned out during the exposure 35 of the material hot to the air.

I find that a more satisfactory way of adding the alkali and of cooling the material when it is taken hot from the boxes is to 40 make a solution of soda ash, or a solution of soda ash and common salt if preferred, and 45 sprinkle the hot material with the solution rather than with the water only. In this way the energizer is carried by the solution 50 into the pores of the carburizing material and so remains in fairly uniform distribution 55 throughout the mass of material; whereas, when the powdered energizer is added to the dry material there is no impregnation and practically no adhesion and the energizer frequently separates from the 60 granular carbonaceous material and settles

as a layer at the bottom of the pile of material, or at the bottom of the pot after packing, thereby making for un-uniform carburization. This defect is overcome by my invention and the cooling of the material 60 and the uniform addition of the energizer is accomplished at one step. I have used this scheme on a large scale, where thousands of uniform parts of low carbon iron have been carbonized and afterward tested and I am 65 convinced that this method of cooling the carburizing material is not only of considerable value as a means of maintaining the material at full strength, but it also is valuable as a means of keeping the material and 70 the work produced uniform. The strength of the solution will vary with the temperature and time in the furnace, and with the degree to which the material is cooled, but I find a satisfactory strength, where soda ash 75 alone is used, to be about ten parts of dry soda ash (sodium carbonate) to one hundred parts of water. Where common salt is also used I prefer to mix seven parts of salt and seven parts of soda ash with one hundred 80 parts of water. This can conveniently be handled in an ordinary sprinkling can; but more elaborate sprinkling devices may be utilized if desired.

The material which I have cooled on a 85 large scale with such a solution of soda ash consisted of small masses (about one-quarter inch in through dimension) made by mixing finely ground coking coal with powdered energizers, coking this mixture and then 90 crushing the resultant coke to produce the small masses above. The solution and method are, however, applicable to other types of carburizing materials. The material is cooled by sprinkling and stirring, 95 with a hoe or shovel, until below a red heat but the sprinkling is not continued so as to leave the material wet. I have found that material which was more or less unsatisfactory when handled in ordinary ways could 100 be maintained highly efficient by the method outlined and the uniformity of the metal parts carburized greatly increased.

What I claim is:

1. The method of maintaining the strength 10 and uniformity of carburizing material which consists in sprinkling the used material, while still hot, with a solution of an energizing material.

2. The method of maintaining the strength 11

and uniformity of carburizing material which consists in sprinkling the used material, while still hot, with a solution of soda ash.

5 3. The method of maintaining the strength and uniformity of carburizing materials, which consists in subjecting the used and hot material to the cooling action of a solution of energizing material.

10 4. The method of uniformly impregnating used carburizing materials, which consists in cooling the used and hot material with a solution of energizing material.

15 5. The method of maintaining the strength and uniformity of carburizing material which consists in subjecting the used and hot material to the cooling action of a solution of soda ash and salt.

6. The method of maintaining the strength

and uniformity of carburizing material, 20 which consists in subjecting hot, used carburizing material to the action of energizing material.

7. The method of uniformly impregnating used carburizing materials, which consists in subjecting hot, used material to a solution of impregnating material for the purpose of cooling the carburizing material and impregnating it with the material in solution.

In testimony whereof, I have hereunto subscribed my name this 13 day of June, 1917.

HUGH RODMAN.

Witnesses:

R. L. KENT,  
ANNA CLOHERTY.